

## UNITED STATES PATENT OFFICE.

ALBERT L. CLAPP, OF DANVERS, MASSACHUSETTS, ASSIGNOR TO THE FLINTKOTE COMPANY, OF BOSTON, MASSACHUSETTS, A CORPORATION OF MASSACHUSETTS.

## WATERPROOFED FIBROUS MATERIAL.

No Drawing.

Application filed October 25, 1920. Serial No. 419,407.

*To all whom it may concern:*

Be it known that I, ALBERT L. CLAPP, a citizen of the United States, residing at Danvers, in the county of Essex and State of Massachusetts, have invented new and useful Improvements in Waterproofed Fibrous Materials, of which the following is a specification.

This invention has for its object, primarily, the waterproofing of fibrous materials, such as felt, paper and other sheet material which is formed in a web by paper-making machinery, but, in addition and perhaps of equal importance, the invention has for its object a method of mechanically precipitating or throwing down a pitch, tar, bitumen, asphalt or other hydrocarbon which forms the disperse phase of an emulsion, of which water forms the continuous phase, so that the bitumen, asphalt or the like may be deposited upon the individual fibers of a fibrous material.

It is now known that bitumen, asphalt, tar and other hydrocarbon oils and pitches, varying greatly in melting point, may be emulsified with water by the use of an emulsifying agent, such as colloidal clay or other colloidal equivalent; and it is also known that such emulsions may be thinned or diluted with water, and may be mixed with fibrous materials in a beating engine, and formed into a sheet or web in a paper-making machine, such as ordinarily employed in the manufacture of felt for roofing purposes. When a sheet is thus formed and is subjected to heat or pressure or both, the bituminous particles coalesce and produce a final product which is to some extent not unlike a sheet of raw felt impregnated or saturated with pitch or bitumen previously liquefied by heat.

I have discovered that it is possible to throw down or precipitate the hydrocarbon or bituminous phase of the emulsion, and to accomplish this while the emulsion is in admixture with the paper stock, so that the hydrocarbon or bitumen is deposited on the individual fibers, and also to cause the particles thereof to stick or adhere to the fibers. Precipitating agents, such as alum or other metal salts which are commonly used in precipitating rosin size or the like in sizing paper have no effect when used alone with an aqueous bitumen emulsion,

but I have found that, if a solution of animal protein is first mixed with the bitumen emulsion, and the precipitating agent is then added, a precipitate is formed which mechanically carries the particles of bitumen and serves as a coagulant therefor.

There are various animal proteins which may be employed. For example, I may use leather, hair, dried fish scraps and the like, all of which, when preliminarily treated with a caustic alkali, form an apparently clear solution. When a precipitant (and I select alum as an example) is added, a flocculent gelatinous precipitate,—in this case, gelatinous aluminium hydrate,—is formed. When this protein solution is added to the aqueous bituminous emulsion, and alum is added, not only is gelatinous aluminium hydrate precipitated, but it also carries down with it the bitumen, all in a flocculent mass. Apparently the gelatinous precipitate acts as an agglutinant or coagulant for the asphalt; but, at any rate, the solid matter is thrown down, leaving a clear liquid above it. If the reaction occurs when the solution and the emulsion (these terms being used principally to distinguish them) are in admixture with the fibrous paper stock, the gelatinous precipitate seems to act as a bond between the fibers and the particles of asphalt.

For exemplifying the production of a suitable animal protein solution, I cite the following. Waste leather, containing little or no grease, and preferably sole leather, is placed in a vat or tank and sufficient water is added to submerge or cover it. The leather scraps are permitted to soak long enough to wet them thoroughly,—say for 15 to 20 minutes. Then to every 100 pounds of leather (dry weight) I add about 12 to 15 pounds of caustic soda (NaOH, 76% basis). The caustic alkali neutralizes the tannic acid and also softens the leather, being in excess of the amount required for neutralization of the acid. After permitting the leather to soak for, say, 15 to 30 minutes, the whole mass is heated and boiled until a liquor is produced which is clear. Such liquor consists of a solution of animal protein, which is of a colloidal nature and which in this case is of a brownish to reddish color. As I have before stated, various other animal proteins may be sub-

stituted for leather, e. g. fish scraps. In fact, casein may be used, although I do not regard it as quite so satisfactory.

In making a sheet of fibrous material, 5 waterpoofed with asphalt or equivalent tar, pitch, bitumen or other hydrocarbon, I proceed as follows, taking an asphalt emulsion as an example. The asphalt emulsion is first prepared, according to the 10 Kirschbraun process, which may be described briefly as follows. Water and clay or equivalent colloid-containing material is first puddled with water to make a paste, and the paste is added to molten asphalt and 15 so mixed therewith as to produce an emulsion in which water constitutes the continuous phase and the clay-asphalt particles the disperse phase. Such an emulsion is non-sticky and may be further thinned and diluted with water.

The animal-protein solution having been prepared, I proceed as follows. I place in a beating engine the desired fibrous materials, such as rags, wood pulp (ground or chemical), sawdust, etc., according to the required 25 specifications of the ultimate product, with sufficient water to ensure the circulation of the mass in the beater tub. This fibrous stock is then beaten and disintegrated to the 30 desired degree of fineness. Then the knives are lifted from the bed plate and the asphalt emulsion is added, the operation of the beater being continued until a homogeneous mixture is secured. The proportion of the 35 asphalt emulsion is varied according to the amount of asphalt which the finished sheet should contain, but, for example, it may be added in the proportion of 300 pounds of asphalt and clay (dry weight) to 1,000 40 pounds of paper stock (dry weight) in the beater.

The animal-protein solution may be added to the paper stock either at the time the raw materials are first introduced into the beater, 45 or when the asphalt emulsion is added, or after the addition of the emulsion, but I prefer to add it coincidently with the addition of the emulsion, so that no additional time is required for its further homogeneous 50 admixture with the paper stock and the emulsion. For 300 pounds of clay and asphalt in the emulsion, sufficient protein solution should be added to represent 100 55 pounds (dry weight) of leather or other animal protein. Preferably the emulsion and the solution are thoroughly mixed before being supplied to the beater. The protein liquor acts to carry the asphalt in uniform suspension throughout the fibrous material.

I now add a precipitant, preferably alum (14% to 16% anhydrous aluminium sulphate) in the proportion of 25 to 30 pounds to 100 pounds of the animal protein (dry weight), and thoroughly incorporate it in 60 the mass in the beater. This is sufficient to

precipitate the protein in the form of a gelatinous aluminium hydrate, which carries the asphalt particles with it, and the composite precipitate is deposited on the fibers uniformly through the mass of paper stock, 70 the gelatinous aluminium hydrate bonding the asphalt to the fibers or causing it to adhere thereto.

The mass of pulp is now ready to be sheeted, and this is accomplished by the use 75 of any suitable form of paper-making machinery such as is employed in the manufacture of raw paper felt, boxboard or the like. The water is removed from the stock according to the usual methods, and the sheet or 80 web is heated and dried. The final product is more satisfactorily waterpoofed than has heretofore been possible, when the asphalt emulsion was incorporated in the fibrous material without precipitation. The gelatinous 85 aluminium hydrate acts not only as an agglutinating agent for the asphalt, to disturb or break down the asphalt emulsion, but it also acts, itself, as a waterpoofing 90 agent.

Some difficulty has heretofore been experienced in sheeting pulp having an asphalt emulsion incorporated therein due to the "balling" of the asphalt particles, as the asphalt is thereby prevented from being uniformly distributed throughout the sheet. When this occurs, the "balls" adhere more or less to the "felts" or blankets of the paper making machine, with the result that 95 the felts or blankets must be frequently 100 cleaned.

By practicing my process as herein described, I obviate largely, if not entirely, these difficulties. The protein solution carries the asphalt particles in suspension and aids in bringing about a more perfect homogeneity in the mixture of pulp and asphalt and prevents the asphalt from balling or agglomerating or coalescing in large particles. While the precipitating agent,—the metal salt—is inert in reference to asphalt, and does not chemically act thereon as a precipitating agent, it does react with the protein solution, the precipitate acting to carry with it the asphalt particles, thereby disturbing or breaking down the emulsion. In the example herein given, the sodium sulphite, resulting from the reaction of the alkaline protein solution with aluminium sulphate, being soluble in water, is removed by 110 the wash water.

What I claim is:

1. The herein described process of breaking down an aqueous bituminous emulsion in which bitumen constitutes the disperse phase which comprises adding thereto an alkaline protein solution, and a precipitating agent capable of reaction with said solution to form a precipitate by which the bituminous particles are thrown down.

2. The herein described process of breaking down an aqueous bituminous emulsion in which bitumen constitutes the disperse phase, which comprises adding thereto an alkaline animal-protein solution and a metal salt capable of reacting with said solution to produce a gelatinous hydrate. 45
3. The herein described process of breaking down an aqueous bituminous emulsion in which bitumen constitutes the disperse phase, which comprises adding thereto an alkaline animal-protein solution and aluminium sulphate whereby a gelatinous aluminium hydrate is precipitated, which acts to throw down the bitumen from the emulsion. 50
4. The herein described process of breaking down an aqueous bituminous emulsion in which bitumen constitutes the disperse phase, which comprises adding thereto an aqueous solution of leather and caustic alkali, and finally a metal salt capable of reacting with said solution to precipitate a gelatinous metal hydrate, which carries with it the bituminous particles. 55
5. The herein described process, which comprises mixing fibrous material, an aqueous bituminous emulsion, and an alkaline protein solution, and then adding a precipitant to form a water-insoluble precipitate from said solution, by which the emulsion is broken down and the bituminous particles deposited on the fibers. 60
6. The herein described process, which comprises mixing fibrous material, an aqueous bituminous emulsion, and an alkaline protein solution, and then adding a precipitant to form a water-insoluble precipitate from said solution, by which the emulsion is broken down and the bituminous particles deposited on the fibers, and finally forming the fibers into a web or sheet. 65
7. The herein described process, which comprises mixing fibrous material, an aqueous bituminous emulsion, and an alkaline solution of animal protein, and then precipitating a gelatinous hydrate from said solution, whereby the bituminous particles are deposited on the fibers. 70
8. The herein described process, which comprises mixing fibrous material, an aqueous bituminous emulsion, and an alkaline leather solution, then adding a metal salt capable of reacting with such solution to precipitate a gelatinous metal hydrate, whereby said emulsion is broken down and the particles of bitumen are deposited on the fibers. 75
9. The herein described process, which comprises mixing fibrous material, an aqueous bituminous emulsion, and an alkaline leather solution, then adding a metal salt capable of reacting with such solution to precipitate a gelatinous metal hydrate, whereby said emulsion is broken down and the particles of bitumen are deposited on the fibers, and finally sheeting said fibrous mass. 80
10. A process comprising mixing fibrous material and an aqueous bituminous emulsion in which the bitumen constitutes the disperse phase, and separately adding reacting ingredients to such mixture to form a precipitating agent by which the bitumen is deposited on the fibers. 85
11. A process, comprising mixing fibrous material, an aqueous bituminous emulsion, and a soluble solution of a body capable of producing a gelatinous precipitate, and then adding a precipitating agent, whereby a gelatinous precipitate is formed and particles of bitumen are deposited on the fibers. 90

In testimony whereof I have affixed my signature.

ALBERT L. CLAPP.